

# United States Patent

Sato et al.

[15] 3,663,209

[45] May 16, 1972

[54] **LIGHT-SENSITIVE SILVER HALIDE  
PHOTOGRAPHIC MATERIAL  
CONTAINING AS A STABILIZER A  
HYDROIMIDAZO-S-TRIAZINE**

[72] Inventors: **Shui Sato; Tomio Nakajima; Masayuki  
Shono, all of Tokyo; Teruo Kagami, Irimi-  
shi, all of Japan**

[73] Assignee: **Konishiroku Photo Industry Co., Ltd.,  
Tokyo, Japan**

[22] Filed: **Dec. 4, 1969**

[21] Appl. No.: **882,311**

[30] **Foreign Application Priority Data**

Dec. 4, 1968 Japan.....43/88338

[52] U.S. Cl.....96/109, 260/239.7

[51] Int. Cl.....G03c 1/34  
[58] Field of Search.....96/109

[56] **References Cited**

**UNITED STATES PATENTS**

2,444,609 7/1968 Heimbach et al.....96/109  
2,444,607 7/1948 Heimbach et al.....96/109

*Primary Examiner*—Norman G. Torchin

*Assistant Examiner*—Richard E. Fichter

*Attorney*—Waters, Roditi, Schwartz & Nissen

[57] **ABSTRACT**

A light-sensitive silver halide photographic material containing in at least one of its photographic layers a hydroimidazo-s-triazine compound as a stabilizer.

**3 Claims, No Drawings**

**LIGHT-SENSITIVE SILVER HALIDE PHOTOGRAPHIC MATERIAL CONTAINING AS A STABILIZER A HYDROIMIDAZO-S-TRIAZINE**

This invention relates to a light-sensitive silver halide photographic material containing in at least one of its photographic layers a hydroimidazo-s-triazine compound as stabilizer, and the object of the invention is to provide a light-sensitive silver halide photographic material which is stable in photographic properties under high temperature and high humidity conditions and is storable for a long period of time.

It has been known that when stored for a long period of time particularly under high temperature and high humidity conditions a light-sensitive photographic material prepared by using a silver halide photographic emulsion generally suffers from such drawbacks that it is decreased or increased in photographic speed and forms the so-called emulsion fog which, after the photographic material has been exposed, brings about the blackening of unexposed portion. The formation of such fog during storage of photographic material and change with time in photographic speed characteristics of photographic emulsion after preparation are not desirable. With an aim to prevent photographic materials from deterioration in photographic properties due to lapse of time or to change of external conditions, stabilizers have heretofore been incorporated into the photographic layers of light-sensitive photographic materials, e.g. emulsion layer, interlayer, sub layer or protective layer. Preferable as such stabilizers, tetrazaindene have been known heretofore. However, the conventional stabilizers are not always satisfactory and tend to cause deterioration of fog, sensitivity and the like photographic properties, during storage under high temperature and high humidity conditions. These drawbacks are obviously undesirable for light-sensitive materials to be used in Japan where high temperature and high humidity are brought about in summer.

In view of such circumstances, we made various studies to find that when a hydroimidazo-s-triazine compound exists in at least one photographic layer of a light-sensitive silver halide photographic material, such as emulsion layer, sublayer, interlayer or protective layer, the light-sensitive photographic material is markedly stable to deterioration in photographic characteristics during storage for a long period of time, particularly during storage under high temperature and high humidity conditions.

Hydroimidazo-s-triazine compounds can be synthesized by isomerization of aziridine rings with sodium iodide and 45 triethylamine hydrochloride or rhodanate disclosed in Journal of the American Chemical Society, Vol. 83, page 2570, and Journal of Organic Chemistry, Vol. 25, page 461, or by dehydrochlorination reaction of  $\beta$ -chloroethylamino groups disclosed in Journal of the American Chemical Society, Vol. 50 77, page 5922. Among such hydroimidazo-s-triazine compounds, those which are particularly useful in the present invention are represented by the following general Formulas I, II, III and IV:

General Formula (I)



General Formula (II)



General Formula (III)



General Formula (IV)



20 (wherein R<sub>s</sub>, which may be same or different groups, represent individually —H, —CH<sub>3</sub> or —C<sub>2</sub>H<sub>5</sub>; R<sub>1</sub> and R<sub>2</sub>, which may be same or different groups, represent individually —OH, —OCH<sub>3</sub>, —SCH<sub>3</sub> or —NH<sub>2</sub>; R<sub>3</sub> represents —H, —NH<sub>2</sub>, —OCH<sub>3</sub> or —OC<sub>2</sub>H<sub>5</sub>; X represents —NH(CH<sub>2</sub>)<sub>n</sub>NH—,

25



or



; and n is an integer of 2 to 6)

30 35 Typical examples of the above-mentioned hydroimidazo-s-triazine compounds employed in the present invention include the following compounds:

(1) 4-hydroxy-2-methoxy-6,7-dihydroimidazo (1,2-a) s-triazine



(2) 2,4-dihydroxy-6,7-dihydroimidazo (1,2-a) s-triazine



(3) 2,4-diamino-6,7-dihydroimidazo (1,2-a) s-triazine



(4) 5-methoxy-2,3,8,9-tetrahydroimidazo (1,2-a:1',2'-c) s-triazine



(5) 5-amino-2,3,8,9-tetrahydroimidazo (1,2-a:1',2'-c) s-triazine hydrochloride



75

(6) 2,8 (or 3,9)-dimethyl-5-ethoxy-2,3,8,9-tetrahydroimidazo (1,2-a:1',2'-c) s-triazine



(7) N,N'-bis (2,3,8,9-tetrahydroimidazo (1,2-a:1',2'-c) s-triazine-5-yl) ethylenediamine



(8) N,N'-bis [2,3,8,9-tetrahydroimidazo (1,2-a:1',2'-c) s-triazine-5-yl] hexamethylenediamine



(9) N,N'-bis [2,3,8,9-tetrahydroimidazo (1,2-a:1',2'-c) s-triazine-5-yl] p-phenylenediamine



(10) N,N'-bis [2,3,8,9-tetrahydroimidazo (1,2-a:1',2'-c) s-triazine-5-yl] piperazine



(11) N,N'-bis [2,8 (or 3,9)-dimethyl-2,3,8,9-tetrahydroimidazo (1,2-a:1',2'-c) s-triazine-5-yl] piperazine



(12) N,N'-bis [2,8 (or 3,9)-diethyl-2,3,8,9-tetrahydroimidazo (1,2-a:1',2'-c) s-triazine-5-yl] trimethylenediamine



(13) 2,3,6,7,10,11-Hexahydrotriamido (1,2-a:1',2'-c:1'', 2''-e) s-triazine



(14) 2,6,10 (or 3,7,11)-trimethyl-2,3,6,7,10,11-hexahydrotriamido (1,2-a:1',2'-c:1'', 2''-e) s-triazine



Concrete synthesis examples of the above-mentioned compounds are shown below.

#### SYNTHESIS EXAMPLE 1

##### Synthesis of the Compound 1

A mixture comprising 5.3 g. of 2-β-chloroethylamino-4,6-dimethoxy-s-triazine, 8.0 cc. of 3.0 N-caustic soda and 22 cc. of ethyl alcohol was boiled for 2 hours, and then the solvent was removed by distillation under reduced pressure. The residual viscous solid was recrystallized two times from water to obtain 1.4 g. of the above-mentioned compound, m.p. 212° C.

Elementary analysis for  $C_8H_8N_4O_2$ :  
 Calculated (%) C: 42.86 H: 4.80 N: 33.32  
 Found (%) C: 42.51 H: 5.10 N: 32.91

#### SYNTHESIS EXAMPLE 2

##### Synthesis of the Compound 5

A mixture comprising 2.7 g. of 2,4-di(β-chloroethylamino-6-chloro-s-triazine, 10 cc. of 28 percent aqueous ammonia solution was reacted for 3 hours in a bath at 90° C., whereby the mixture once became a transparent solution but soon formed a white precipitate. After cooling the liquid, the precipitate was recovered by filtration and was extracted with hot water. Thereafter, the extract was combined with the filtrate, and the mixed liquid was concentrated under reduced pressure and was cooled to deposit a crystalline mass. The mass was recovered by filtration and was recrystallized from water to obtain 0.5 g. of the above-mentioned compound, m.p. 250° C.

Elementary analysis for  $C_8H_{11}ClN_6$ :  
 Calculated (%) C: 39.20 H: 5.13 N: 39.2 Cl: 16.60  
 Found (%) C: 38.87 H: 5.17 N: 39.17 Cl: 16.64

#### SYNTHESIS EXAMPLE 3

##### Synthesis of the Compound 8

To a solution of 1.0 g. of the corresponding tetraethyleneimino compound in 30 cc. of chloroform was added a solution of 0.7 g. of sodium iodide in 20 cc. of acetone, and the mixed solution was allowed to stand at room temperature for 12 hours to deposit a crystalline mass. The mass was recovered by filtration, was washed with acetone and was then recrystallized from water to obtain 0.7 g. of the above-mentioned compound, m.p. above 250° C.

Elementary analysis for  $C_{20}H_{30}N_{12} \cdot 2H_2O$ :  
 Calculated (%) C: 50.61 H: 7.22 N: 35.42  
 Found (%) C: 50.24 H: 7.21 N: 35.22

#### SYNTHESIS EXAMPLE 4

##### Synthesis of the Compound 13

A solution of 3.0 g. of triethylene melamine and 1.5 g. of sodium iodide in 150 cc. of acetone was allowed to stand at room temperature for 24 hours to deposit a needle-like crystalline mass. The mass was recovered by filtration, was washed with acetone and was then recrystallized from water to obtain 2.3 g. of the above-mentioned compound, m.p. above 250° C.

Elementary analysis for  $C_9H_{12}N_6\frac{1}{2}H_2O$ :

|                |          |         |          |
|----------------|----------|---------|----------|
| Calculated (%) | C: 50.70 | H: 6.15 | N: 39.41 |
| Found (%)      | C: 51.15 | H: 6.24 | N: 39.82 |

## SYNTHESIS EXAMPLE 5

## Synthesis of the Compound 14

A mixture comprising tripropylene melamine synthesized from cyanuric chloride and propylene imine, sodium iodide and acetone was treated in the same manner as in Synthesis Example 4 to obtain the above-mentioned compound in the form of white solid.

Elementary analysis for  $C_{12}H_{18}N_6$ :

|                |          |         |          |
|----------------|----------|---------|----------|
| Calculated (%) | C: 58.52 | H: 7.37 | N: 34.12 |
| Found (%)      | C: 58.09 | H: 7.42 | N: 34.33 |

Other hydroimidazo-s-triazine compounds than those mentioned above can also be synthesized according to the above-mentioned synthesis examples.

The thus obtained hydroimidazo-s-triazine compounds should be present in the photographic layers of light-sensitive photographic materials according to any procedures for incorporating conventional photographic stabilizers into the layers of the constituents. For example, the present compound may be added to a photographic emulsion in the form of a solution in a suitable inorganic or organic solvent such as a mixed solution of water and a lower alcohol, a lower alcohol, dimethyl sulfoxide or the like. The present compound may be added at any time during the step for preparation of photographic emulsion, and may be previously incorporated into the starting materials for preparation of the emulsion. Generally, however, it is preferable and is most effective to add the compound after completion of the second aging.

The emulsion to be used for preparation of the present photographic material may have been subjected to noble metal sensitization, sulfur sensitization, sensitization with al-

graphic stabilizers not only for monochromatic photographic materials but also for color photographic materials.

The amount of the hydroimidazo-s-triazine compound to be added to or incorporated into the photographic layers of a light-sensitive photographic material varies depending not only on the kind of the compound but also on the kind of the emulsion employed, i.e. whether the emulsion is silver chloride, silver bromide or silver iodide, the content of the solid solution, the particle size and photographic sensitivity of the silver halide emulsion, and the desired degree of stabilization. Generally, however, the compound is added in an amount of about 0.01-8 g. per mole of silver halide.

The following examples illustrate the present invention, but the invention is not limited thereby and various modifications are possible within the scope of the invention.

## EXAMPLE 1

A neutral negative silver iodobromide emulsion containing 5 mole percent of silver iodide was charged with a gold sensitizer and was subjected to second ripening, and the thus treated emulsion was divided into six portions. One portion of the emulsion was coated, as it was, onto a support to prepare a control sample. Another portion was charged with an aqueous solution of 30 mg. per 0.035 mole of said silver halide of the known stabilizer 4-hydroxy-6-methyl-1,3,3a,7-tetrazaindene, and was coated onto a support to prepare a comparative sample. The other four portions were individually charged with methanol solutions of the compounds set forth in Table 1 in such amounts as shown in the table, and were coated onto supports to prepare samples of the present invention. These samples were subjected to ordinary sensitometry according to the JIS method K-7604 to obtain the results as set forth in Table 1. The photographic speed was shown in terms of a relative value calculated by assuming as 100 the speed of the control sample immediately after coating.

TABLE 1

| Sample                          | Stabilizer                    | Amount added (mg.) | Immediately after coating |                | After incubation at 55° C. for 3 days |                | After incubation at 50° C. and humidity of 80% for 3 days |                |
|---------------------------------|-------------------------------|--------------------|---------------------------|----------------|---------------------------------------|----------------|-----------------------------------------------------------|----------------|
|                                 |                               |                    | Fog                       | Relative speed | Fog                                   | Relative speed | Fog                                                       | Relative speed |
| Control sample                  |                               |                    | 0.13                      | 100            | 0.62                                  | 81             | 0.34                                                      | 110            |
| Comparative Sample              | Above-mentioned tetrazaindene | 30                 | 0.13                      | 100            | 0.12                                  | 94             | 0.08                                                      | 80             |
|                                 | Compound (1)                  | 20                 | 0.12                      | 100            | 0.10                                  | 98             | 0.10                                                      | 101            |
| Sample of the present invention | Compound (7)                  | 40                 | 0.11                      | 97             | 0.12                                  | 100            | 0.12                                                      | 98             |
|                                 | Compound (10)                 | 35                 | 0.10                      | 103            | 0.12                                  | 102            | 0.11                                                      | 101            |
|                                 | Compound (13)                 | 30                 | 0.11                      | 100            | 0.12                                  | 97             | 0.12                                                      | 99             |

kylene oxide polymer or the like chemical sensitization, optical sensitization or super color sensitization. The hydroimidazo-s-triazine compounds of the present invention do not injure the photographic speed attained by said sensitization and inhibit the increase of fog generated thereby, with the result that the resulting photographic materials can be more effectively enhanced in light-sensitivity increase due to said sensitization, and can be prevented from lowering in photographic speed and increase in fog during storage, particularly under high temperature and high humidity conditions.

In preparing the light-sensitive silver halide photographic materials of the present invention, the above-mentioned compounds in accordance with the present invention may be used, without any detrimental interactions, in combination with other photographic additives, e.g. other stabilizers, coating aids, hardeners, toners, matting agents and the like.

Further, in the case of color photographic materials containing in the emulsion layers thereof large amounts of color formers or containing dispersions of color formers dispersed as protective colloids by use of high boiling oil or low boiling oil or the mixture of both, the compounds of the present invention can inhibit the generation of color fog due to fog of silver halide emulsions, and hence are effective as photo-

55 As is clear from Table 1, it is understood that the light-sensitive silver halide photographic materials of the present invention show markedly excellent stability in fog and speed, and have such properties that they are less in desensitization under high temperature and high humidity conditions than the known stabilizer.

## EXAMPLE 2

60 The same photographic emulsion as in Example 1 was subjected to second ripening and was incorporated according to an ordinary procedure with the color former, 1-(4'-phenoxy-3'-sulfonylphenyl)-3-heptadecyl-5-pyrazolone, to prepare a color photographic emulsion. This emulsion was divided into 65 three portions. One portion of the emulsion was coated, as it was, onto a support to prepare a control sample. The other two portions were individually charged with methanol solutions of 30 mg. and 40 mg. per 0.035 mole of said silver halide of the present Compound 8, and were coated onto supports to 70 prepare samples of the present invention. These samples were exposed by means of a sensitometer, were developed with a color developing solution composed mainly of diethyl-p-phenylenediamine, and were subjected to ordinary bleaching, fixing and water-washing treatments. The results were as shown 75 in Table 2.

TABLE 2

| Sample                          | Stabilizer   | Amount added (mg.) | Immediately after coating |                | After incubation at 55° C. for 3 days |                | After incubation at 50° C. and humidity of 80% for 3 days |                |
|---------------------------------|--------------|--------------------|---------------------------|----------------|---------------------------------------|----------------|-----------------------------------------------------------|----------------|
|                                 |              |                    | Fog                       | Relative speed | Fog                                   | Relative speed | Fog                                                       | Relative speed |
| Control sample                  |              | 0.12               | 100                       | 0.26           | 95                                    | 0.19           | 96                                                        |                |
| Sample of the present invention | Compound (8) | 35                 | 0.11                      | 99             | 0.12                                  | 102            | 0.11                                                      | 103            |
|                                 | do           | 54                 | 0.10                      | 97             | 0.10                                  | 100            | 0.09                                                      | 99             |

As is clear from the above table, the light-sensitive photographic materials according to the present invention were markedly excellent in fog and photographic speed particularly under high temperature and humidity conditions, and could give excellent color images without any color fog.

What we claim is:

1. A light-sensitive silver halide photographic element comprising at least one photographic layer containing 0.01-8 g./mole of silver halide of a hydroimidazo-s-triazine compound, having one of the following general Formulas I, II, III and IV



15



(IV)

20 wherein Rs, which may be same or different groups, represent individually —H, —CH<sub>3</sub> or —C<sub>2</sub>H<sub>5</sub>; R<sub>1</sub> and R<sub>2</sub>, which may be same or different groups, represent individually —OH, —OCH<sub>3</sub>, —SCH<sub>3</sub> or —NH<sub>2</sub>; R<sub>3</sub> represents —H, —NH<sub>2</sub>, —OCH<sub>3</sub> or —OC<sub>2</sub>H<sub>5</sub>; X represents —NH(CH<sub>2</sub>)<sub>n</sub>NH—,

25 (I)



30 or



(II)

35 ; and n is an integer of 2 to 6.

2. A light-sensitive silver halide element as claimed in claim 1, wherein said element is a light-sensitive silver halide color photographic element.

3. A light-sensitive silver halide photographic element as claimed in claim 2, wherein said photographic layer is an emulsion layer, interlayer, sublayer or protective layer.

\* \* \* \* \*

45

50

55

60

65

70

75